

## UNITED STATES PATENT OFFICE

2,290,859

## BENEFICIATION OF LUBRICANTS

Robert E. Burk and Everett C. Hughes, Cleveland Heights, Ohio, assignors to The Standard Oil Company, Cleveland, Ohio, a corporation of Ohio

No Drawing. Application April 13, 1940,  
Serial No. 329,523

8 Claims. (Cl. 252—49)

Where a lubricating oil is subjected to drastic high temperature usage, as for instance in an internal combustion engine, it tends to change in viscosity and lubricating activity. The mechanism of the change is obscure and involves complex factors. By some writers the action has been ascribed to oxidation. However, the matter is not so simple as this, and the degradation can be brought about in the absence of oxygen. We have now found that by subjecting an oil to the action of certain material, the degradation tendency of the oil in drastic high temperature usage is arrested, the material however, although very effective, has a side action of *prima facie* making the oil corrosive on metal surfaces which it lubricates, but as a part of the invention this undesired side tendency is corrected and controlled by conjoined action of another material which we have found particularly to bring about such results; and the lubricant as a whole is thus of outstanding advantage for severe high temperature usage.

To the accomplishment of the foregoing and related ends, the invention, then, comprises the features hereinafter fully described, and particularly pointed out in the claims, the following description setting forth in detail certain illustrative embodiments of the invention, these being indicative however, of but a few of the various ways in which the principle of the invention may be employed.

In accordance with the invention, an oil of lubricating viscosity, high or low in accordance with the particular duty intended, and for instance being in general of 45 to 200 viscosity Saybolt Universal at 210° F., is subjected to the action of a small amount of a very active agent maintaining the oil against viscosity change in degradation change otherwise occurrent, and the side effect of corrosive action on metals with which the oil is contacted, is controlled by also providing a metal corrosion inhibiting agent. The material for treating the oil is phosphorus, of the ordinary or yellow form, and it is effective in quantities of 0.001—0.25 per cent, greater amounts being unnecessary, and in particular we have found that amounts of 0.01—0.05 per cent are satisfactory. The amount of the metal corrosion inhibiting agent similarly can be small, for instance 0.001—5 per cent, and generally amounts less than 2 per cent are satisfactory. The metal corrosion inhibiting agent is an organic ester or thioester of a phosphorus acid, i. e. phosphorus and phosphoric acids, such esters having the general formula



wherein R is an alkyl, aryl, alkaryl or cycloparaffin 60

hydrocarbon, Z is hydrogen or alkyl or aryl hydrocarbons or mixtures thereof, X is oxygen or sulphur, and M is phosphorus or phosphorus monoxide. Such compounds for instance as tricresyl phosphite, tricresyl phosphate, tricresyl thiophosphate, tributyl phosphate, etc. are particularly desirable.

As an example: In an oil of 350 viscosity Saybolt Universal at 100° F., there is incorporated 0.025 per cent of ordinary phosphorus, and 0.15 per cent of tricresyl phosphite. This lubricant run in a test at 350° F. for 42 hours shows a viscosity of 381, lacquer formation 2.1 Mg, and appearance rating B minus, whereas the oil without the addition agents and run at the same temperature for the same length of time changes in viscosity to 479, and lacquer formation is 7.9, and the appearance rating C plus.

As another example: In a lubricating oil of 20 Mid-Continent stock and having a gravity 389 Saybolt Universal at 100° F., there is incorporated 0.05 per cent of ordinary phosphorus and 0.15 per cent of tricresyl phosphite. This lubricant run in test at 350° F. for 42 hours shows a viscosity 403, lacquer formation 4.2 Mg, and appearance rating C, whereas the oil without the addition agents and tested at the same temperature and for the same length of time changed in viscosity to 630 and showed lacquer formation 46.3 Mg, and appearance rating E minus.

As another example: In a similar lubricating oil as in the immediately preceding example, there is incorporated 0.025 per cent of ordinary phosphorus and 0.15 per cent of tricresyl phosphate. This lubricant run in a similar test as in the foregoing, showed viscosity 474, lacquer formation 18.3, and appearance rating B minus.

It was suggested many years ago, to add inactive or red phosphorus to transformer-filling oils with the idea of checking sludging. No measures were taken against metal corrosion. And, so far as we are aware it has not been known to treat oil with an active agent otherwise occasioning corrosion of metal surfaces, and at the same time guard such metal against untoward action.

Other modes of applying the principle of the invention may be employed, change being made as regards the details described, provided the features stated in any of the following claims, or the equivalent of such, be employed.

We therefore particularly point out and distinctly claim as our invention:

1. A process of increasing the durability of mineral oils of lubricating viscosity in high temperature usage, which comprises subjecting the oil to the action of a small amount of phosphorus and inhibiting metal corrosion of the phosphorus by a small amount of tricresyl phosphite.

2. A process of increasing the durability of

mineral oils of lubricating viscosity in high temperature usage, which comprises subjecting the oil to the action of a small amount of phosphorus and inhibiting metal corrosion of the phosphorus by a small amount of tricresyl phosphate.

3. A process of increasing the durability of mineral oils of lubricating viscosity in high temperature usage, which comprises subjecting the oil to the action of a small amount of phosphorus and inhibiting metal corrosion of the phosphorus by a small amount of tricresyl thiophosphate.

4. A process of increasing the durability of mineral oils of lubricating viscosity in high temperature usage, which comprises subjecting the oil to the action of a small amount of phosphorus and inhibiting metal corrosion of the phosphorus by a small amount of an ester of a phosphorus acid from the group consisting of phosphorus and phosphoric acids.

5. A lubricant comprising a mineral oil of lubricating viscosity, and a small amount of phosphorus and a small amount of tricresyl phosphite.

6. A lubricant comprising a mineral oil of lubricating viscosity, and a small amount of phosphorus and a small amount of tricresyl phosphate.

7. A lubricant comprising a mineral oil of lubricating viscosity, and a small amount of phosphorus and a small amount of tricresyl thiophosphate.

8. A lubricant comprising a mineral oil of lubricating viscosity, and a small amount of phosphorus and a small amount of an ester of a phosphorus acid having the general formula



wherein R is an alkyl, aryl, alkaryl or cycloparaffin hydrocarbon, Z is hydrogen or alkyl or aryl hydrocarbons or mixtures thereof, X is oxygen or sulphur, and M is phosphorus or phosphorus monoxide.

ROBERT E. BURK.  
EVERETT C. HUGHES.